

1,357,920.

H. ABRAHAM,  
COMPOSITION ROOFING,  
APPLICATION FILED JULY 26, 1917.

Patented Nov. 2, 1920.

*Fig. 1*



*Fig. 2*



Inventor

Herbert Abraham.

By his Attorney

Lester W. Dillenbeck

# UNITED STATES PATENT OFFICE.

HERBERT ABRAHAM, OF NEW YORK, N. Y., ASSIGNOR TO STANDARD PAINT COMPANY,  
A CORPORATION OF NEW JERSEY.

## COMPOSITION ROOFING.

1,357,920.

Specification of Letters Patent. Patented Nov. 2, 1920.

Application filed July 26, 1917. Serial No. 182,872.

To all whom it may concern:

Be it known that I, HERBERT ABRAHAM, a citizen of the United States, and a resident of the borough of Manhattan, in the city, county, and State of New York, have invented certain new and useful Improvements in Composition Roofings, of which the following is a full, clear, and exact specification.

My invention relates to a composition roofing material containing bituminous matter. The object of my invention is to provide a roofing material which possesses greater durability, and yet can be manufactured with comparatively less expense than the present forms of felt composition roofing on the market. The product herein described and claimed is adapted to be used in sheet or in shingle form.

0 The essential feature of the invention consists in combining a comparatively thick layer of bituminous matter containing a small proportion by weight of loose fibers, and a foundation sheet of felted fibrous fabric saturated with asphalt.

In the accompanying drawings illustrating my invention, Figure 1 is a cross-section of a sheet of roofing material embodying my invention, and Fig. 2 a sectional view of a modified form.

Referring to the drawings, 1 indicates a felted fibrous sheet (commonly known as "roofing felt") saturated with asphalt or other suitable bituminous composition; 2 is a comparatively thick layer of bituminous material containing non-felted fibers; and 3 is a bituminous coating free from fibers applied in a comparatively thin layer to the upper surface of the roofing, and 4 represents a similar coating which may or may not be applied to the lower surface of the roofing.

A coating 5 (Fig. 2) of powdered, granulated or angular mineral matter, may be applied to one or both surfaces of the finished product, or as an alternative, coating 3 may be made in accordance with the disclosure of my Patents Nos. 775,635 and 775,636 granted on November 22, 1904, that 50 is having a colored pigment mixed therein to impart a permanent color.

In practice I have found that it is desirable to incorporate approximately 10% to 20% of fibers in the bituminous matter constituting layer 2. The fibers may be of

animal, vegetable, or mineral origin, consisting of disintegrated felt or paper stock, slag-wool, asbestos or similar materials. The loose fibers are disseminated throughout the bituminous matter and form a homogeneous mass therewith.

In manufacturing the roofing I take a sheet of ordinary roofing felt and saturate it with the melted bituminous composition in the usual manner. To the saturated felted sheet I apply a layer of bituminous substance of a comparatively high melting point containing fibers. This layer is first spread on loosely, preferably while in a heated state, and then compressed by passing through steel rollers or otherwise under pressure to compact it into a tough and resilient mass.

The product is more weather-resisting than ordinary prepared roofing of the same thickness, composed of a felted fabric saturated and coated with bituminous compositions and for the following reasons: It is well recognized in the art, that although felt fibers impart strength to the finished product, they nevertheless constitute the weakest part from the viewpoint of weather-resistance. They must therefore be thoroughly protected or inclosed by the bituminous constituents. Saturating the felt alone will not enable it to withstand satisfactorily the effects of the weather, as the fibers on the surface will soon rot, and by capillarity or otherwise, carry moisture into the center of the sheet, so that a progressive disintegrative action takes place. The saturated felt is therefore ordinarily safe-guarded by an additional layer or coating of bituminous matter. This surface-coating constitutes the main protection against the inroads of the weather. As long as it remains intact, the felt fibers can retain their strength. When it is oxidized or worn away by attrition of the elements, so as to uncover the felt fibers, the roofing will soon perish. It has therefore been stated correctly that a felt roofing is no more durable than its weather coating.

Attempts have been made to increase the durability of the weather coating by spreading it on in a thicker layer. Bituminous materials least susceptible to temperature changes, and having the greatest ductility, such as certain blown petroleum asphalts, fatty acid pitches, mixtures of asphaltites

and residual fluxes, etc., with and without the addition of finely divided mineral fillers, have been tried for this purpose. It was found, either that at low temperatures or 5 upon aging the thick coatings become hard and brittle and cracked on bending, or else during the hot summer weather or in the tropics, the thick coating softened to such an extent that it checked or ran, or easily 10 became distorted upon being subjected to unusual pressure.

I have found that the addition of non-felted fibers to the thick layer of bituminous coating overcomes these defects. As the 15 non-felted fibers are stirred into the melted bituminous matter, the latter loses its fluidity, and becomes converted into a plastic mass which can no longer be melted—even at high temperatures, but which can 20 nevertheless be molded or formed under pressure.

Whereas the fibers in the felted sheet even under the most favorable conditions, cannot be made to carry more than 1 to 1½ times its weight of bituminous matter, it is 25 a surprising fact that when the non-felted fibers are added to the bituminous matter, not more than ½ to ¼ its weight of fibers can be incorporated. In other words, whereas a 30 sheet of felted fibers saturated with bituminous matter carries between 40 and 50% by weight of fibers, the maximum weight of non-felted fibers which can be incorporated in a mixture with bituminous matter, ranges 35 between 12½ and 20% of the total. This phenomenon may be explained by the fact that non-felted fibers occupy much greater bulk than an equal weight of the same fibers in the felted state.

40 I have found further that a thick coating of bituminous matter containing non-felted fibers is less brittle at low temperatures and is not as liable to crack on bending as an equally thick coating composed of the same 45 bituminous matter without further additions. This is probably due to the fact that the non-felted fibers disseminated throughout the bituminous matter bind the mass to-

gether, similar to the reinforcing metal in concrete, thereby imparting greater strength and toughness to the composition.

On account of the smaller percentage of fibers present in a coating of this nature, it is accordingly less acted upon by the weather than a felted sheet of the same kind 5 of fibers saturated with bituminous matter of similar character. Although it is not entirely necessary, yet it is advisable to further protect the non-felted fibers in the coating (2) by applying to its weather-surface 6 a comparatively thin coating of bituminous matter free from fibers.

Roofing made in accordance with the foregoing disclosure will present the maximum proportion of bituminous matter to the 61 action of the weather, and carry the bulk of the fibers at the bottom of the sheet, where they are most efficiently protected. A smaller percentage of fibrous matter will be required in manufacturing the roofing of a 70 given thickness or weight per unit area, than would be the case if a felted fibrous sheet was employed as at present. Since the fibers are relatively more expensive than the bituminous matter, the improved process 75 will result in considerable economy.

The material may be manufactured and sold in sheet form, or if desired, the sheet may be cut into shingles of the required size. I have found that shingles cut from 80 the said sheet are tougher and stiffer than those manufactured in the usual manner.

Various modifications and changes may be made in the construction herein above described without departing from the scope 85 of my invention.

What I claim as my invention and desire to secure by Letters Patent is:

A composition roofing comprising a layer 90 of felt saturated with bituminous matter, and a compacted coating layer consisting of bituminous matter containing not over twenty per cent., by weight, of non-felted fibrous material, said coating layer being thicker than the felt layer.

HERBERT ABRAHAM.